

# UNITED STATES PATENT OFFICE.

GEORGE B. BRADSHAW, OF ROSELLE PARK, NEW JERSEY.

## PROCESS OF MAKING PICRIC ACID.

1,168,266.

Specification of Letters Patent. Patented Jan. 11, 1916.

No Drawing.

Application filed November 8, 1915. Serial No. 60,279.

To all whom it may concern:

Be it known that I, GEORGE B. BRADSHAW, a citizen of the United States of America, residing at Roselle Park, in the county of Union and State of New Jersey, have invented certain new and useful Improvements in Processes of Making Picric Acid, of which the following is a specification.

This invention relates to a process of making picric acid, and in its more intense aspect deals with the treatment of para-phenol-mono-sulfonic acid.

One of the objects of the present invention is to produce picric acid, preferably obtained by nitrating or otherwise treating certain phenol sulfonic acids.

Another object is to provide a simple and practical process for making picric acid which may be carried out in a shorter time and at less expense than processes heretofore proposed.

A further object is to provide a reliable, safe and efficient process for manufacturing a higher grade of picric acid.

Other objects will be in part obvious and in part hereinafter pointed out.

The invention accordingly consists in the several steps and the relation and order of one or more of those steps with relation to each of the others thereof which will be exemplified in the hereinafter disclosed process and the scope of the application of which will be indicated in the claims that follow.

While it may have been attempted to treat simultaneously certain phenolic bodies such as ortho- and para-phenol-mono-sulfonic acids for the production of picric acid, such processes have required a relatively large amount of time and expense, and it is believed that these objections, among others, may be fully overcome by nitrating the phenolic body, when all of the phenol is in the form of para-phenol-mono-sulfonic acid.

The process may be carried out in its mechanical aspect in numerous ways known to those familiar with the subject and the following may be cited as a preferable example: One part of phenol is first sulfonated with about 15% more sulfuric acid of about 93% strength than theoretically required to form phenol-sulfonic acid and the resulting mixture of ortho- and para-mono-sulfonic acids is all substantially changed to para-mono-sulfonic acid by diluting with water till the mixture is about 30° Bé, and then boiling with live steam thoroughly. A hun-

dred gallon batch may be boiled three hours. The resulting dilute solution of para-phenol-mono-sulfonic acid of about 20° Bé, is then gradually added to three and one-half parts of nitric acid of about 40° Bé during which the temperature should be kept relatively low. After the reaction subsides the mixture is heated to a temperature of about 200° F. until the reaction has completely occurred. The mass is then allowed to settle and cool, and the picric acid crystallizes out and is removed in the usual way.

A second method is to change the ortho sulfonic into para sulfonic by heating to 260° F. with excess sulfuric acid while stirring. This procedure would be used where metal nitrating vessels are employed and all dilution of acid must be avoided.

It is thus seen that this invention produces a desirable, simple, practical and inexpensive process of making picric acid and is believed to accomplish, among others, all of the objects, and advantages herein set forth.

As many changes could be made in carrying out the above process without departing from the scope of the invention, it is contended that all matter contained in the above description shall be regarded as illustrative and not in a limiting sense.

I claim as my invention:

1. The herein described process of producing picric acid comprising the steps of converting phenol completely into para-phenol sulfonic acid and nitrating said para-phenol sulfonic acid.

2. The herein described process of producing picric acid comprising the step of nitrating substantially pure para-phenol-mono-sulfonic acid.

3. The herein described process of producing picric acid comprising the step of nitrating substantially pure para-phenol-mono-sulfonic acid and completing the nitrination by the application of heat.

4. The herein described process of producing picric acid comprising the steps of converting phenol into substantially pure para phenol sulfonic acid in the presence of water so as to form a dilute solution thereof, mixing three and one-half parts of nitric acid of about 40° Bé with one part of said solution, heating the mixture until the reaction is completed, and allowing the picric acid to crystallize out of the reactive mass.

5. The herein described process of producing picric acid which consists in sulfonating

phenol to produce a mixture of phenol-  
mono-sulfonic acids, diluting the mixed sul-  
fonic acids with water and boiling the same  
with steam to convert the same into aqueous  
5 solution of substantially pure para-mono-  
sulfonic acid, mixing the said solution with  
nitric acid and then finally heating the same  
to a temperature of approximately 200° F.

after which the picric acid is allowed to  
crystallize.

In testimony whereof I affix my signature  
in the presence of two witnesses.

GEORGE B. BRADSHAW.

Witnesses:

CLARENCE CHURCHILL,  
JAMES HARPER.